

C. E. RAHR,  
ROOFING ELEMENT,  
APPLICATION FILED OCT. 17, 1918.

1,340,347.

Patented May 18, 1920.



Inventor:

Chester E. Rahr

By Knight, Brown, Murphy & May  
Attorneys

# UNITED STATES PATENT OFFICE.

CHESTER E. RAHR, OF BROOKLINE, MASSACHUSETTS, ASSIGNOR TO THE FLINTKOTE COMPANY, OF BOSTON, MASSACHUSETTS, A CORPORATION OF MASSACHUSETTS.

## ROOFING ELEMENT.

1,340,347.

Specification of Letters Patent. Patented May 18, 1920.

Application filed October 17, 1918. Serial No. 258,523.

To all whom it may concern:

Be it known that I, CHESTER E. RAHR, a citizen of the United States, residing at Brookline, in the county of Norfolk and 5 State of Massachusetts, have invented new and useful Improvements in Roofing Elements, of which the following is a specification.

This invention has relation to roofing materials and has for its object to provide certain improvements therein.

The invention consists of a roofing element; that is, a sheet or shingle in which the asphalt-saturated fibrous foundation has 15 on its upper and lower sides or faces coated and uncoated parallel zones, the coated zone of one face overlying or underlying, as the case may be, the uncoated zone of the other face. Each coated zone is less than one-half 20 the width of the element so as to provide a middle zone which is uncoated on each face.

Preferably each coating consists of a layer of asphalt, pitch or like material of relatively high melting point, in which is embedded or with which is interlocked a surface layer. The surface layer preferably 25 consists of grit, *i. e.* crushed mineral such as slate. For the two faces, slate of different colors or shades may be employed, so 30 that, reversing the sheet, one or the other color may be exposed in laying the roof covering. In lieu, however, of forming both surface layers of grit, one of them may consist of sheet asbestos, which, like crushed 35 slate, serves as a fire-retardant, or some other sheet material.

For many purposes it is desired that at least a portion of each sheet shall be left uncoated so as to expose the rough face 40 of the saturated felt, as in laying built-up roofings of the character of those illustrated in the application of William A. Harris, Serial No. 259,090, filed on the 21st day of October, 1918.

45 Referring to the accompanying drawings,—

Figure 1 represents a portion of a sheet of roofing embodying the invention, said sheet being illustrated in conventional form.

50 Fig. 2 illustrates a shingle which embodies the invention.

Fig. 3 is a conventional view illustrating how the sheet shown in Fig. 1 may be wound into a roll of minimum diameter.

Fig. 4 represents a roll in longitudinal 55 section.

The body of the roofing element, whether it be a sheet or a shingle, consists of felt, preferably rag felt or equivalent fibrous material, which is saturated with a relatively 60 low-melting-point pitch or asphaltum, or other equivalent waterproofing compound, such as used in the manufacture of commercial roofing felts.

On the drawing, this fibrous foundation 65 is indicated conventionally at *a*. This saturating compound is applied to the foundation by drawing a sheet of felt through a saturating tank in which the compound is maintained at the desired degree of fluidity 70 by the application of heat, the excess or surplus compound being expressed from the sheet by squeeze rolls, thereby leaving the face of the sheet rough with the surface fibers more or less exposed. Upon the lower 75 portion of the upper face or side of the sheet, there is applied by any suitable instrumentality, such as a coating roller, a layer *b* of higher-melting-point pitch or asphalt,—preferably blown asphalt having 80 a melting point sufficiently high so that the asphalt will not be affected by solar heat. This layer *b* covers a zone of the sheet between the edges thereof, which zone is less than one-half of the width of the sheet. A 85 similar layer *c* of pitch or asphalt is applied to the under side or face of the sheet, but is located below or under the uncoated zone *d* of the top face. This coating *c* is likewise in width less than one-half of the 90

width of the sheet *a*, so that, between the inner edge *e* of the upper coating *b* and the inner edge *f* of the lower layer or coating *c* there is a zone *g* of the sheet parallel with and intermediate the upper and lower edges 95 thereof which is uncoated on both faces. While these coatings *b* and *c* are soft and plastic, I embed therein surface layers of crushed mineral, preferably crushed slate, as indicated at *h* and *i* respectively. By 100 forming these two layers *h* and *i* of slate of different or contrasting colors or tints it is possible for the user to so lay the sheet or element as to expose the layer of the desired color, or to lay the sheets to form 105 bands of different colors.

In some instances, instead of a fire-resist- 110 ant layer of crushed mineral *i*, I may sub-

stitute a sheet of asbestos in lieu thereof, this asbestos being locked to the foundation *a* by the layer *c* of asphaltum. Or, if desired, I may substitute a sheet of heavy canvas or 5 burlap or other fabric which will increase the strength of the roofing when laid.

In Fig. 2, I have shown a roofing shingle, having the same construction as that described except that naturally it is of the 10 proper dimensions.

Assuming that the sheet in Fig. 1, between its upper and lower edges, is thirty-two inches in width, each coated zone is preferably fifteen inches in width, leaving an intermediate zone of two inches on which 15 there is no coating on either face. These same relative proportions are preserved preferably in a shingle, which of course is of smaller dimensions, say nine by sixteen 20 inches. By having the uncoated zone *g*, it is possible to coil the sheet into a roll of minimum diameter, the uncoated zone of each convolution bending so as to permit the convolutions to assume the shape shown in Fig. 25 3. The shingles may be packed in a compact package, by reason of the zone *g* to accomplish a practically like result.

Having thus explained the nature of my 30 said invention, what I claim is:—

1. A roofing element comprising a fibrous asphalt-impregnated foundation having its opposite faces coated with asphaltic material in zones, parallel with the top and bottom edges thereof, with fire-resistant material, the coated zone of one face being opposite the uncoated zone of the other face.

2. A roofing element comprising a fibrous asphalt-impregnated foundation having an intermediate zone which is uncoated on 35 either face thereof, and having upper and lower zones of which one is coated with a

surfacing material on one face and the other is coated on the opposite face.

3. A roofing element comprising a fibrous asphalt-impregnated foundation, one side 45 of said foundation being provided with an asphaltic coating which covers only the lower portion thereof and the other side being provided with a coating which covers only the upper portion, said coatings being 50 surfaced with mineral material.

4. A roofing element comprising a fibrous asphalt-impregnated foundation, one side of said foundation being provided with a coating which covers only the lower portion 55 thereof and the other side being provided with a coating which covers only the upper portion, each of said coatings being fire-resistant.

5. A roofing element comprising a fibrous 60 asphalt-impregnated foundation, one side of said foundation being provided with a coating which covers only the lower portion thereof and the other side being provided with a coating which covers only the 65 upper portion, each of said coatings comprising a layer of asphalt and a surface layer of crushed mineral embedded therein.

6. A roofing element comprising a fibrous asphalt-impregnated foundation, one side of 70 said foundation being provided with a coating which covers only the lower portion thereof and the other side being provided with a coating which covers only the upper portion, each of said coatings comprising a 75 layer of asphalt and a surface layer of crushed mineral embedded therein, the said minerals being different in color or tint.

In testimony whereof I have affixed my signature.

CHESTER E. RAHR.